

[54] **SILVER HALIDE PHOTOGRAPHIC ELEMENT CONTAINING AN ACETYLENE SULFONYL COMPOUND AS HARDENER**

[75] Inventors: Tomio Nakajima, Tokyo; Sadao Sugita, Hanno; Yukichi Kishida; Masabumi Yoshimoto; Noboru Ishida, all of Tokyo, Japan

[73] Assignee: Konishiroku Photo Industry Co., Ltd.; Sankyo Company Limited, both of Tokyo, Japan

[22] Filed: **June 21, 1971**

[21] Appl. No.: **155,237**

[30] **Foreign Application Priority Data**

June 20, 1970 Japan ..... 45/53612

[52] U.S. Cl. .... **96/67, 96/76 R, 96/109, 96/111, 260/117, 106/125, 117/62.2**

[51] Int. Cl. .... **G03c 1/76, G03c 1/48, G03c 1/34, G03c 1/30**

[58] **Field of Search** ..... 96/111, 109, 50, 96/67, 76 R; 260/117; 106/125; 117/62.2

[56] **References Cited**  
UNITED STATES PATENTS  
3,505,071 4/1970 Emmi ..... 96/111  
2,816,125 12/1957 Allen et al. ..... 96/111 X

FOREIGN PATENTS OR APPLICATIONS  
1,193,290 5/1970 Great Britain ..... 96/111

*Primary Examiner*—J. Travis Brown  
*Assistant Examiner*—Won H. Louie, Jr.  
*Attorney*—Eric H. Waters et al.

[57] **ABSTRACT**  
Acetylene sulfonyl compounds of the formula R—C≡C—(CH<sub>2</sub>)<sub>n</sub>—SO<sub>2</sub>—R' wherein R, R' and n are defined in claims are found to be useful as hardeners for the gelatin films of light-sensitive silver halide photographic materials. Synthesis and use of these compounds also are disclosed.

**6 Claims, No Drawings**

SILVER HALIDE PHOTOGRAPHIC ELEMENT  
CONTAINING AN ACETYLENE SULFONYL  
COMPOUND AS HARDENER

This invention relates to a hardener for the gelatin 5 films of a light-sensitive silver halide photographic material, said hardener comprising a compound of the general formula,



wherein R' is a lower alkyl group or a phenyl or alkyl- 10 phenyl group; R is a hydrogen atom, a lower alkyl group or a phenyl, alkylphenyl, alkoxyphenyl or halo- phenyl group; and n is zero or 1.

Generally, a light-sensitive silver halide photographic material is prepared by forming various layers such as 15 silver halide photographic emulsion layer, filter layer, inter layer, protective layer, sub layer, backing layer, etc. on a suitable support such as glass, paper or synthetic resin film. These layers are composed mainly of gelatin, so that the physical properties of said layers are dependent chiefly upon the physical properties of gelatin. However, gelatin itself is low in melting point, water-swelling and low in mechanical strength, and these properties are not desirable, or rather to say, are fatal drawbacks for the layers constituting a light-sensitive 20 silver halide photographic material.

In view of the above, many attempts have heretofore been made to improve the physical properties of gelatin by treatment with various hardeners. These hardeners, however, have such photographic defects as being 25 strong in desensitizing action and high in fog-forming action and, in the case of color photographic emulsions, bring about such drawbacks that they disturb the color developability of couplers or are too vigorous in hardening action to make the production of light-sensitive photographic materials difficult. Further, due 30 particularly to the recent tendency of quick development and the adoption of automatic developing machines, the physical properties of films have come to be required more strong.

We made extensive studies on hardeners capable of giving gelatin films having such strong physical properties as to be suitable for the above-mentioned quick and automatic treatment of light-sensitive photographic materials to find that acetylene sulfones having the aforesaid general formula display excellent hardening actions without deteriorating the properties of photographic materials.

Examples of the compounds having the aforesaid 35 general formula are as follows:

1. Ethyl 1-pentylnyl sulfone



b.p. 96-97°C/  
10<sup>-3</sup>mmHg

2. Phenyl 1-propynyl sulfone



m.p. 68-69°C

3. p-Tolyl 1-propynyl sulfone



m.p. 96-98°C

4. Phenyl 2-propynyl sulfone



55

60

65

m.p. 93°C

5. p-Tolyl 2-propynyl sulfone



m.p. 95-97°C

6. Phenyl 2-butynyl sulfone



m.p. 63.5°C

7. Methyl phenylethynyl sulfone



m.p. 66-67°C

8. p-Tolyl phenylethynyl sulfone



m.p. 80-81°C

9. p-Tolyl p-tolylethynyl sulfone



b.p. 154-155°C/  
10<sup>-4</sup>mmHg

10. p-Tolyl p-bromophenylethynyl sulfone



m.p. 107-108°C

11. p-Tolyl m-methoxyphenylethynyl sulfone



b.p. 165-167°C/  
10<sup>-4</sup>mmHg

12. Phenyl 3-phenyl-2-propynyl sulfone



m.p. 116-117°C

The above-mentioned compounds may be synthesized by oxidizing corresponding acetylene sulfides according to, for example, the method disclosed in Bull. Soc. Chim. Fr., 1966, 3024. Procedures for synthesis of the compounds are set forth below as reference examples.

REFERENCE EXAMPLE 1

To a solution of 7.53 g of ethyl 1-pentylnyl sulfide in 100 ml. of methylene chloride is added a 0° to 5°C. a solution of 48.8 g of m-chloroperbenzoic acid in 400 ml. of methylene chloride, and the resulting mixture is stirred at 0° to 5°C. for 4 hours. The reaction mixture is diluted with 1.0 l. of ether, and the dilution is washed with a saturated aqueous sodium bicarbonate solution and water in this order and then dried with anhydrous sodium sulfate. Subsequently, the solvent is removed by distillation, and the residue is subjected to distillation under highly reduced pressure to obtain 5.11 g of ethyl 1-pentylnyl sulfone, yield 54.3%, b.p. 96°-97°C./-10<sup>-3</sup>mmHg.

## REFERENCE EXAMPLE 2

To a solution of 40.2 g of 1-propynyl p-tolyl sulfide in 600 ml. of glacial acetic acid is added 33.8 g of 30% hydrogen peroxide, and the resulting mixture is heated at 50° to 60°C. for 2 hours. The reaction mixture is poured into 5 liters of ice water, and deposited crystals are recovered by filtration to obtain 42.4 g of p-tolyl 1-propynyl sulfone in the form of prisms, yield 88.2%, m.p. 90°-91°C.

The compound having the aforesaid general formula may be incorporated as a gelatin film hardener into any of gelatin-containing layers constituting a light-sensitive photographic material, e.g. the sub layer, emulsion layer, inter layer, protective layer and backing layer, whereby the film can be hardened. Alternatively, a photographic film bearing the above-mentioned layers may be hardened by immersing the film in a solution of the said compound, or by dipping the film in any of the baths containing the said compound at the time of development treatment. The hardener of the present invention may be used in combination with a known inorganic hardener such as chromium alum or chromium trichloride, or a known organic hardener such as formalin, glyoxal, acrolein or the like.

In incorporating into the gelatinous layers of a light-sensitive silver halide photographic material, the hardener of the present invention is used ordinarily in the form of a solution in water or methanol, but may also be used in the form of a solution in one or more of organic solvents such as dimethylformamide and the like. The amount of the hardener to be incorporated is preferably in the range of 1 to 20% by weight based on the weight of gelatin in the coating liquid. In case the hardener is desired to be incorporated into a light-sensitive silver halide emulsion layer, it is preferable to incorporate the hardener after the second ripening of said silver halide emulsion. In this case, the hardener of the present invention may be used in combination with other ordinary additives for said photographic emulsion such as, for example, stabilizers, coating aids, sensitizers or sensitizing dyes. Further, the photographic emulsion used may have been subjected to chemical sensitization by use of gold or sulfur, and may have been incorporated with a coupler.

When applied in the above manner to a light-sensitive silver halide photographic material, the hardener of the present invention displays excellent hardening effect without adversely affecting the fog, sensitivity and the like photographic properties of the photographic emulsion. Further, even if the light-sensitive photographic material incorporated with the hardener is stored for a long period of time, the hardener provides effective stability without giving any detrimental effect to the photographic emulsion, and exhibits excellent hardening effect even when the photographic material is subjected to high temperature development and automatic treatment.

The present invention is illustrated in further detail below with reference to examples, but it is needless to say that the invention is not limited only to these, and various modifications are possible within the scope of the invention.

## EXAMPLE 1

A silver iodobromide emulsion for photographic negative, which emulsion contains 3 mole% of silver iodide was charged with a gold sensitizer and then subjected to second ripening. Subsequently, the emulsion was divided into 4 portions, and one portion was coated as it was on a support to prepare a control sample, while the remaining 3 portions were individually incorporated with each of methanol solutions of the previously exemplified compounds (2), (7) and (10) and then coated on a support to prepare samples of the present invention.

These samples were individually stored at 55°C. for 3 days, and at 50°C. and RH 80% for 3 days. The thus stored samples and the fresh samples (which were immediately after coating on supports) were individually immersed in pure water, and the temperature at which each sample was dissolved on the film surface was measured. On the other hand, the stored samples were immersed in a 3% solution of sodium carbonate monohydrate at 50°C., and the time required for each sample to initiate the dissolution of its film surface was measured. Further, the samples were subjected to sensitometry to measure the values of relative speed and fog of the photographic emulsions. The results obtained were as set forth in Table 1.

TABLE 1

| Sample                                             | Amount of hardener per 10 g. of gelatin (mg.) | Hardening characteristics               |                |                           |                                                          |                                              |                           |                                                              |                                              |
|----------------------------------------------------|-----------------------------------------------|-----------------------------------------|----------------|---------------------------|----------------------------------------------------------|----------------------------------------------|---------------------------|--------------------------------------------------------------|----------------------------------------------|
|                                                    |                                               | Sensitivity characteristics of emulsion |                |                           | Temperature required for dissolution in pure water (°C.) |                                              |                           | Time required for initiation of dissolution in alkali (sec.) |                                              |
|                                                    |                                               | Fog                                     | Relative speed | Immediately after coating | After storage at 55°C. for 3 days                        | After storage at 50°C. and RH 80% for 3 days | Immediately after coating | After storage at 55°C. for 3 days                            | After storage at 50°C. and RH 80% for 3 days |
| Control sample                                     |                                               | 0.20                                    | 100            | 31                        | 32                                                       | 34.4                                         | 1.8                       | 1.9                                                          | 2.0                                          |
| Sample incorporated with exemplified compound (2)  | 300                                           | 0.16                                    | 98             | (a)                       | (a)                                                      | (a)                                          | 130                       | 180                                                          | 210                                          |
| Sample incorporated with exemplified compound (7)  | 300                                           | 0.15                                    | 96             | (a)                       | (a)                                                      | (a)                                          | 91.0                      | 200                                                          | 600                                          |
| Sample incorporated with exemplified compound (10) | 300                                           | 0.17                                    | 98             | 60                        | (a)                                                      | (a)                                          | 75.0                      | 165                                                          | 168                                          |

\* Above 65.

As is clear from the above table, the samples according to the present invention had no desensitizing action, successfully inhibited the fog and displayed excellent hardening effects.

## EXAMPLE 2

The same photographic emulsion as in Example 1 was subjected to second ripening and then charged with a color coupler 1-(4'-phenoxy-3'-sulfophenyl)-3-heptadecyl-5-pyrazolone. Thereafter, the emulsion was divided into 4 portions, and one portion was coated as it was on a support to prepare a control sample, while the remaining 3 portions were individually incorporated with each of aqueous solutions of the previously exemplified compounds (3), (6) and (11) and then coated on supports to prepare samples of the present invention.

These samples were individually measured to determine hardening effect in the same manner as in Example 1. Further, the samples were subjected to sensitometry by developing the samples with a color developer containing diethyl-p-phenylenediamine and effecting ordinary bleaching, fixing and water-washing treatments. The results obtained were as set forth in Table 2, in which the speed is represented by a relative speed.

## EXAMPLE 3

A high speed light-sensitive silver iodobromide emulsion for roentgenography, which contained 3 mol % of silver iodide was subjected to ordinary chemical ripening, and then charged with 100 ml. per liter of the emulsion of 5-methyl-7-hydroxy-s-triazolo(2.5-a)pyrimidine as a stabilizer and 2 g per liter of the emulsion of saponin as a coating aid. Subsequently, the emulsion was divided into seven portions, and one portion was coated as it was on a cellulose triacetate support to prepare a control sample, while the remaining six portions were individually coated to prepare samples of the present invention.

These samples were exposed according to the method regulated in Japanese Industrial Standards, subjected to high temperature quick development at 30°C. for 1 minute and 30 seconds, at 35°C. for 40 seconds, and at 40°C. for 25 seconds by use of a strongly alkaline roentgen film-developing solution containing 1-phenyl-3-pyrazolidone and hydroquinone, and then measured in speed and fog. Further, the sample were measured in hardening effects according to the same procedures as in Example 1.

Separately, the films were measured in surface strength in the following manner: Each sample was dipped for 2 minutes in a 3% sodium carbonate (mono-

TABLE 2

| Sample                                             | Amount of hardener per 10 g. of gelatin (mg.) | Sensitivity characteristics of emulsion (immediately after preparation) |                | Hardening characteristics |                                   |                                              |                           |                                   |                                              |
|----------------------------------------------------|-----------------------------------------------|-------------------------------------------------------------------------|----------------|---------------------------|-----------------------------------|----------------------------------------------|---------------------------|-----------------------------------|----------------------------------------------|
|                                                    |                                               |                                                                         |                | Pure water bath (° C.)    |                                   |                                              | Alkali bath (sec.)        |                                   |                                              |
|                                                    |                                               | Fog                                                                     | Relative speed | Immediately after coating | After storage at 55°C. for 3 days | After storage at 50°C. and RH 80% for 3 days | Immediately after coating | After storage at 55°C. for 3 days | After storage at 50°C. and RH 80% for 3 days |
| Control sample                                     |                                               | 0.06                                                                    | 100            | 32                        | 38                                | 42                                           | 2.0                       | 2.5                               | 3.2                                          |
| Sample incorporated with exemplified compound (3)  | 250                                           | 0.04                                                                    | 105            | 56                        | (a)                               | (a)                                          | 95                        | (b)                               | (b)                                          |
| Sample incorporated with exemplified compound (6)  | 250                                           | 0.03                                                                    | 98             | 63                        | (a)                               | (a)                                          | 122                       | 280                               | (b)                                          |
| Sample incorporated with exemplified compound (11) | 250                                           | 0.04                                                                    | 96             | 68                        | (a)                               | (a)                                          | 92                        | (b)                               | (b)                                          |

<sup>a</sup> Above 65. <sup>b</sup> Above 300.

As is clear from Table 2, the samples according to the present invention displayed excellent hardening effects without injuring the photographic properties. Moreover, not only the couplers used were not injured in color development but also no dye stains were observed.

hydrate) solution at 50°C. Immediately thereafter, the film was wiped and then scratched with a pin (R: 3 mm.). The film surface strength is expressed in terms of a load (g) with which the film surface had begun to be scratched with the pin.

The results obtained were as set forth in Table 3.

TABLE 3

| Sample                                             | Characteristics of emulsion            |                                 |                                 |                                                              | Hardening characteristics                       |                                                   |                                    |                           | Film surface strength              |                                    |
|----------------------------------------------------|----------------------------------------|---------------------------------|---------------------------------|--------------------------------------------------------------|-------------------------------------------------|---------------------------------------------------|------------------------------------|---------------------------|------------------------------------|------------------------------------|
|                                                    | Developed at 30° C. for 1 min. 30 sec. | Developed at 33° C. for 40 sec. | Developed at 40° C. for 25 sec. | Time required for initiation of dissolution in alkali (sec.) | Load with which scratch began to be formed (g.) | After storage at 50° C. and R.H. 80±10 for 3 days | After storage at 55° C. for 3 days | Immediately after coating | After storage at 55° C. for 3 days | After storage at 55° C. for 3 days |
| Control sample                                     | 100                                    | 0.12                            | 100                             | 0.18                                                         | 100                                             | 0.22                                              | 28                                 | 45                        | 56                                 | 5                                  |
| Sample incorporated with exemplified compound (2)  | 250                                    | 0.09                            | 110                             | 0.16                                                         | 120                                             | 0.19                                              | 150                                | (*)                       | 30                                 | 20                                 |
| Sample incorporated with exemplified compound (3)  | 250                                    | 0.11                            | 105                             | 0.16                                                         | 110                                             | 0.20                                              | 142                                | (*)                       | 30                                 | 120                                |
| Sample incorporated with exemplified compound (6)  | 250                                    | 0.08                            | 100                             | 0.14                                                         | 105                                             | 0.17                                              | 170                                | (*)                       | 30                                 | 120                                |
| Sample incorporated with exemplified compound (7)  | 250                                    | 0.07                            | 100                             | 0.15                                                         | 100                                             | 0.17                                              | 180                                | (*)                       | 50                                 | 146                                |
| Sample incorporated with exemplified compound (12) | 250                                    | 0.10                            | 108                             | 0.18                                                         | 115                                             | 0.18                                              | 120                                | (*)                       | 20                                 | 150                                |
|                                                    |                                        |                                 |                                 |                                                              |                                                 |                                                   |                                    |                           |                                    | 170                                |
|                                                    |                                        |                                 |                                 |                                                              |                                                 |                                                   |                                    |                           |                                    | 130                                |

\* Above 300.

60

65

55

45

40

35

As is clear from the above table, the samples incorporated with the hardeners of the present invention effectively inhibit fog even at the time of high temperature quick development, and display excellent hardening effects without any detrimental influence on speed of the emulsion. Moreover, they are high in film surface strength and do not undergo any mechanical damage even when subjected to automatic developing machines.

## 10 What we claim is:

1. A light-sensitive silver halide photographic material comprising (1) a support, (2) at least one gelatin layer coated on said support, one of said layers containing the silver halide and (3) from 1 to 20% by weight of the gelatin in any of said layers of a hardener which is a compound having the formula  

$$R-C\equiv C-(CH_2)_n-SO_2-R'$$
 wherein R' is a lower alkyl, phenyl or alkylphenyl group; R is a hydrogen atom, a lower alkyl, phenyl, alkylphenyl, alkoxyphenyl or halophenyl group; and n is zero or 1.
2. The material according to claim 1 wherein R is methyl, R' is phenyl and n is zero.
- 25 3. The material according to claim 1 wherein R is methyl, R' is p-tolyl and n is zero.
4. The material according to claim 1 wherein R is methyl, R' is phenyl and n is 1.
5. The material according to claim 1 wherein R is phenyl, R' is methyl and n is zero.
- 30 6. The material according to claim 1 wherein R is m-methoxyphenyl, R' is p-tolyl and n is zero.

\* \* \* \* \*